

May 2, 1950

O. HEDLUND

2,505,896

CONSTRUCTION OF COMPOSITE METAL ARTICLES

Filed April 22, 1944



Fig. 1



Fig. 5



Fig. 2



Fig. 6



Fig. 3



Fig. 7



Fig. 4



INVENTOR.  
OSCAR HEDLUND

*Joseph P. Teagno  
Attorney*

## UNITED STATES PATENT OFFICE

2,505,896

## CONSTRUCTION OF COMPOSITE METAL ARTICLES

Oscar Hedlund, Battle Creek, Mich., assignor to Eaton Manufacturing Company, Cleveland, Ohio, a corporation of Ohio

Application April 22, 1944, Serial No. 532,263

6 Claims. (Cl. 29—156.7)

1

This invention relates to the construction of composite metal articles and more particularly to the fabrication of composite metallic poppet valves for internal combustion engines.

It is the usual practice due to the corrosive and/or erosive effect of the combined high temperatures and lead oxide generated in the combustion of high octane fuels to coat and overlay the valve seat and outer surface of the valve head with an alloy of the composition of 80% nickel and 20% chromium to thereby resist the destructive action of the combustive gases and prolong the life of the valves.

Heretofore, this coating or overlaying of the valve head and/or seat has been applied by means of an electric or gas welding process with the result that it proved slow and consequently costly. Furthermore, in so applying this metal, it was almost impossible to obtain a coating or overlaying of uniform thickness; it being particularly desirable to obtain an article having uniform thickness of nickel-chromium alloy without surface porosity and with uniform cohesion between the metals to be bonded together.

The stem of that portion of the valve head not directly contacted by the combustive gases is ordinarily made of a comparatively inexpensive metal having extreme high tensile strength characteristics at elevated temperatures; such an alloy comprises .40 to .50% carbon; .30 to .80% silicon; a maximum of .70% manganese; 13.00 to 15.00% each of chromium and nickel; .20 to 5.0% molybdenum; 1.75 to 3.00% tungsten; a maximum of .03% each of phosphorus and sulphur; and the balance of iron.

An object of the invention is to provide a method of making a composite metallic poppet valve in a less expensive and speedier method.

Another object of the invention is to provide a method of producing a composite metallic article having a substantially uniform coating of heat corrosion and/or erosion resistant metal.

Another object of the invention is to provide a valve having a head and valve seat coated or overlayed with a coat of heat corrosion and/or erosion resistant metal, said metal being effectively bonded to the stem of the valve.

A further object of the invention is to provide a composite valve having a head, seat, and stem of dissimilar metals effectively bonded together with uniform cohesion throughout their juncture.

A still further object of the invention is to provide a method of bonding dissimilar metals together comprising assembling the metals in juxtaposed relationship; inserting the metals in

5 a container in the presence of an inert gas; sealing the metals within the container; heating the assembly to a predetermined temperature and then forging the assembly so as to provide a bond between the metals.

And yet, another object of the invention is to provide a method of making a composite metallic valve comprising preforming a number of dissimilar metallic members; assembling the 10 members in complementary relationship; inserting the members in a metallic container in the presence of an inert gas; sealing the container; heating the container and members to a suitable forging temperature; forging the container and members so as to provide a welding of the 15 metals throughout their complementary surfaces; removing the container from the members, and then forging the members so as to produce a valve having an exposed head of one metal, a 20 valve seat of another metal, and stem of still another metal, all effectively bonded together.

Other objects and advantages of the invention will appear from the following description taken in connection with the drawings forming 25 a part of the specification, and which:

Figure 1 is a side elevational view of a pair of cylindrical members adapted to be welded together;

Figure 2 is a longitudinal sectional view of 30 the members in assembly within a sealed container;

Figure 3 is a longitudinal sectional view of the members after initial forging and removal of the containers;

35 Figure 4 is a longitudinal sectional view of the members after the second forging operation;

Figure 5 is a longitudinal sectional view of the members after subsequent forging and piercing operations;

Figure 6 is a fragmentary longitudinal sectional view of the completed article;

Figure 7 is a longitudinal elevational view of a modified form of the invention similar to Figure 2; and

45 Figure 8 is a fragmentary longitudinal view of the completed article forming the modification of the invention.

Referring to the drawings for more specific details of the invention, 10 represents a cylindrical body member adapted to be welded to a cylindrical disk member 12. The body member 10 is made of metal possessing high tensile characteristics at elevated temperatures, whereas disk 12 is composed of a heat corrosion and/or erosion resistant metal.

In the process of bonding members 10 and 12 together, the complementary surfaces of the members are initially ground and thoroughly cleaned so as to provide smooth mating surfaces free of dirt or other foreign matter. The members are next assembled in juxtaposed relationship and inserted in a container 14 in the presence of an inert gas. A cover plate 16 is then placed upon the container and welded or otherwise suitably secured thereto so as to hermetically seal the members within the container. By so sealing the members in the container in the presence of an inert gas, oxidation of the surfaces to be bonded is materially reduced with the result that a more effective and uniform weld is possible between the members. The contained assembly is then heated to a suitable predetermined temperature and initially forged so as to provide for a uniform bonding of the members 10 and 12 throughout their juncture. The container and cover are next removed from the forged members in any suitable manner so as to provide an assembly as indicated in Figure 3.

After the completion of the initial forging operation the assembly is further forged and machined in accordance with the teachings of the patent to McBride, No. 1,984,751 to thus provide a finished bimetallic valve 18 as indicated by Figure 6.

In a modified form of the invention, 100 represents a cylindrical body member having an enlarged head 102 and an annular recess portion 104 adapted to have bonded thereto a disk 106 and a ring 108. The cylindrical member is preferably made of metal possessing high tensile strength characteristics at elevated temperatures, and the disk and ring are made of heat corrosion and/or erosion resistant metal.

In the assembling of the members to be bonded together, the disk 106 is placed upon the enlarged head 102 in juxtaposed relationship thereto; and the ring 108 is slipped over the body of the cylindrical member 100 and placed in complementary relationship to the underside of the head adjacent the recess 104.

The assembly is then inserted in a container 110 complementary in shape to the assembly and is sealed therein in the presence of an inert gas by a cover 112 welded or otherwise suitably secured to the container.

The assembly and container are then heated and forged in a manner similar to the preferred embodiment of the invention with the resultant production of an article or valve 114 shown by Figure 8.

While this invention has been described in connection with certain specific embodiments, the principle involved is susceptible of numerous other applications that will readily occur to persons skilled in the art. The invention is, therefore, limited only as indicated by the scope of the appended claims.

What I claim is:

1. The method of making a composite metallic poppet valve comprising preforming a cylindrical body member; preforming a disk member complementary to the head of the body member; preforming a ring having a part complementary to a portion of the body member; assembling the members in complementary relationship with the disk and ring in annular axial abutting relationship to one another and arranged juxtaposed the head of the body member on opposite sides thereof; inserting the members in a thin walled container in the presence of an inert gas; seal-

ing the members within the container; heating the container and members to a predetermined forging temperature; forging the container and members as a unit so as to provide for welding of the members one to another; removing the container from the bonded assembly further forging the composite structure to desired valve form and machining the valve to completion.

2. The method of making a composite metallic poppet valve comprising preforming a cylindrical body member possessing high tensile strength characteristics; preforming a heat corrosion and/or erosion resistant disk member complementary to the head of the body member; preforming a ring of physical and chemical properties similar to the disk member having a part complementary to a portion of the body member; assembling the members in complementary relationship with the disk and ring in annular axial abutting relationship to one another and arranged juxtaposed the head of the body member on opposite sides thereof; inserting the members in a thin walled container in the presence of an inert gas; sealing the members within the container; heating the container and members to a predetermined forging temperature; forging the container and members as a unit so as to provide for welding of the members one to another; removing the container from the bonded assembly further forging the composite structure to desired valve form and machining the valve to completion.

3. The method of making a composite metallic poppet valve comprising preforming a cylindrical body member possessing high tensile strength characteristics at elevated temperatures; preforming a disk member of 80-20 nickel-chromium complementary to the head of the body member; preforming a ring of similar constituency as the disk member having a part complementary to a portion of the body member; assembling the members in complementary relationship with the disk and ring in annular axial abutting relationship to one another and arranged juxtaposed the head of the body member on opposite sides thereof; inserting the members in a thin walled container in the presence of an inert gas; sealing the members within the container; heating the container and members to a predetermined forging temperature; forging the container and members as a unit so as to provide for welding of the members one to another; removing the container from the bonded assembly further forging the composite structure to desired valve form and machining the valve to completion.

4. The method of making a valve for internal combustion engines having a mushroom shaped head, a stem integral therewith and a coating of protective material welded upon the head and seat of the valve comprising; preforming a metallic disk member; preforming an annular metallic ring member; preforming a cylindrical cone-shaped metallic member; inserting the members in abutting position in a thin walled sheet metallic container in the presence of an inert gas with the ring in annular axial abutting relationship upon the disk with a portion of the cylindrical member disposed therebetween; hermetically sealing the container with the members enclosed with the inert gas; heating the container and contents to predetermined temperature; forging the container and contents to provide for the bonding of the members together across the abutting surfaces of the members whereby two of the members afford a protective

coating for the other member; removing the container from the forged welded members; further forging the members so as to provide a valve having a mushroom shaped head composed of the three members, two members coating the head and a stem integral therewith composed of the member that is coated.

5. The method of making a valve for internal combustion engines having a mushroom shaped head, a stem integral therewith, a coating of protective metal welded upon the head, and a coating of another protective metal welded upon the seat of the valve comprising; preforming a metallic member adapted to provide the head protective coating for the valve; preforming a second metallic member adapted to provide the protective coating for the seat of the valve; preforming a third metallic member adapted to provide the mushroom shaped head and integral stem of the valve; inserting the members in proper abutting relationship with the first and second metallic members in end abutting relationship to one another and juxtaposed the mushroom-shaped head of the third metallic member on opposite sides thereof in a thin metallic container in the presence of an inert gas; hermetically sealing the container with the members enclosed with the inert gas; heating the container and contents to predetermined temperature; forging the container and contents to provide for the bonding of the members together across the abutting surfaces of the members whereby two of the members afford a protective coating upon the third member; removing the container from the forged welded members; further forging the members so as to provide a valve having a mushroom shaped head composed of the three members, one member coating the head, the second member coating the seat and the third member forming the base, head and integral stem of the valve.

6. A method of making a composite metallic article comprising preforming a cylindrical body

member; preforming a disk member complementary to the head of the body member; preforming a ring having a part complementary to a portion of the body member; assembling the members in complementary relationship with a disk and ring in annular axial abutting relation to one another and arranged juxtaposed the head of the body member on opposite sides thereof; inserting the members in a thin walled metallic container in the presence of an inert gas; hermetically sealing the members within the container; heating the container and members to a predetermined forging temperature; forging the container and members as a unit so as to provide for the welding of the members one to another; and then removing the container from the welded assembly.

OSCAR HEDLUND.

#### REFERENCES CITED

The following references are of record in the file of this patent:

#### UNITED STATES PATENTS

| Number    | Name      | Date          |
|-----------|-----------|---------------|
| 242,194   | Fleitman  | May 31, 1881  |
| 340,223   | L'Epine   | Apr. 20, 1886 |
| 673,525   | Martin    | May 7, 1901   |
| 726,026   | Canda     | Apr. 21, 1903 |
| 1,355,234 | Lachman   | Oct. 12, 1920 |
| 1,374,110 | Pittevil  | Apr. 5, 1921  |
| 1,658,925 | Jardine   | Feb. 14, 1928 |
| 1,948,793 | Lewis     | Feb. 27, 1934 |
| 1,956,818 | Acre      | May 1, 1934   |
| 2,002,641 | McBride   | May 28, 1935  |
| 2,052,862 | Armstrong | Sept. 1, 1936 |
| 2,059,584 | Johnson   | Nov. 3, 1936  |
| 2,123,416 | Graham    | July 12, 1938 |
| 2,178,527 | Wellman   | Oct. 31, 1939 |

#### FOREIGN PATENTS

| Number  | Country       | Date          |
|---------|---------------|---------------|
| 487,464 | Great Britain | June 21, 1938 |